

# UNITED STATES PATENT OFFICE.

WILLIAM FRIESE-GREENE, OF LONDON, ENGLAND.

## PANCHROMATIC SENSITIZING COMPOSITION.

1,383,620.

Specification of Letters Patent.

Patented July 5, 1921.

No Drawing.

Application filed July 8, 1919. Serial No. 309,455.

To all whom it may concern:

Be it known that I, WILLIAM FRIESE-GREENE, a subject of the King of England, residing in London, England, have invented 5 certain new and useful Improvements in Panchromatic Sensitizing Composition, of which the following is a specification.

The invention provides an improved color sensitizing for the preparation of panchromatic plates whereby enhanced color effects 10 may be obtained. A part of the invention also consists in the method of making up this sensitizing.

A specific object of the invention is to improve color photography processes based 15 upon the employment of two colors whereby an approximation to natural color effects is obtained. In particular the invention aims at improving two-color cinematography.

20 These and other objects and features of the invention will now be described in detail.

The color sensitizing according to the present invention comprises pinacyanol, pinaverdol, pinachrome, flavazine (sometimes flava- 25 zin or flavasine) and ammonia mixed with water, and preferably the proportions employed are as follows:—

|    |                 |           |
|----|-----------------|-----------|
| 30 | Pinacyanol      | 2 grains. |
|    | Pinaverdol      | 6 grains. |
|    | Pinachrome      | 2 grains. |
|    | Flavazine       | 4 grains. |
|    | Ammonia (.880)  | 4 ozs.    |
| 35 | Distilled water | 65 pints. |

In making up the sensitizing the first four ingredients in the quantities stated are preferably placed in 10 ozs. of boiling alcohol and stirred for say 10 minutes until thor- 40oughly dissolved, after which 65 pints of distilled water may be added at a tem- 40perature of about 70° Fahr. and then the 4 ozs. of ammonia added. The film or plate to be color-sensitized is immersed in this mix- 45ture for about 5 minutes and kept constantly in movement. The drying should be effected quickly at a temperature of about 75° Fahr.

The light sensitive surface of a photo- 50graphic plate or film color-sensitized by this formula is panchromatic, and such plates or films may be used for any purpose for which panchromatic plates or films are suitable, giving very efficient results and satisfactory color effects. According to the present in- 55 vention, however, panchromatic plates or films, color-sensitized by the above formula,

are used in improving color-photography on the two-color principle.

The ingredients detailed above are referred to by the names commonly given to them in the chemical and color photographic industry. It will be understood, however, that pinacyanol (sometimes known as sensitol red) is obtained by treating quinaldinium salts with formaldehyde followed by alkali. 65 Pinaverdol is p-toluquinaldinquinolinium-methylcyaninbromid.

Pinachrome is p-ethoxyquinaldin-p-methoxyquinolinethylcyaninebromid.

Flavazine is one of the few important 70 dyes belonging to the small class of pyrazolone dye-stuffs and is a dye similar to tartrazin.

The marked difference of color values ob- 75 tained by the use of the special sensitizer aforesaid, leaves room for considerable ma- 80nipulation of the colors in the toning- or staining-bath, so that the depth of color of either plate may be modified as required to obtain a proper balance according to the 85 color effects desired and according to the subject under treatment. This balance can only be judged by the operator for each sub- 90ject, and will depend largely upon individual taste, but the fact that a large differ- 95ence of color value is obtained by means of this invention leaves scope for the desired manipulation.

What I claim as my invention and desire 90 to secure by Letters Patent is:—

1. A color sensitizing for color-photogra- 95phy comprising pinacyanol, pinaverdol, pin- 100achrome, flavazine and ammonia mixed with water.

2. A color sensitizing for color-photogra- 95phy comprising the following substances in substantially the proportions indicated:

|                 |           |     |
|-----------------|-----------|-----|
| Pinacyanol      | 2 grains. |     |
| Pinaverdol      | 6 grains. | 100 |
| Pinachrome      | 2 grains. |     |
| Flavazine       | 4 grains. |     |
| Ammonia (.880)  | 4 ounces. |     |
| Distilled water | 65 pints. |     |

3. A method of making up a color sensi- 105tizer for color-photography, comprising placing pinacyanol, pinaverdol, pinachrome and flavazine in boiling alcohol, stirring until dissolved and adding water and ammonia.

4. A method of making up a color sensi- 110tizer for color-photography, comprising

placing pinacyanol, pinaverdol, pinachrome and flavazine in boiling alcohol, stirring them until dissolved and then adding water at a temperature of 70° F. and ammonia.

5 5. A method of making up a color sensitizer for color-photography consisting in placing 2 grains of pinacyanol, 6 grains of pinaverdol, 2 grains of pinachrome, and 4

grains of flavazine in 10 ounces of boiling alcohol, stirring for ten minutes until thoroughly dissolved, adding 65 pints of distilled water at a temperature of 70° F. and finally adding 4 ounces of ammonia (.880.)

In testimony whereof I affix my signature.

WILLIAM FRIESE-GREENE.